

# United States Patent Office

2,974,021

Patented Mar. 7, 1961

1

2,974,021

## PROCESS AND COMPOSITION FOR CHEMICALLY TREATING TITANIUM AND ITS ALLOYS

Albert Borowik, Bridgeport, Pa., assignor to the United States of America as represented by the Secretary of the Army

No Drawing. Filed Feb. 8, 1957, Ser. No. 639,121

8 Claims. (Cl. 41—42)

(Granted under Title 35, U.S. Code (1952), sec. 266)

The invention described herein may be manufactured and used by or for the Government for governmental purposes without the payment of any royalty thereon.

This invention relates to a material and process for the chemical polishing and etching of titanium and its alloys for metallographic examination and has for an object to provide a suitable reagent and process for this purpose.

An examination of the true microstructure of a metal specimen has been said to be the prime function of chemical as distinguished from electrolytic polishing. The specimen may have been mechanically polished beforehand to obtain good light-reflective surface. Chemical etching dissolves more metal at grain boundaries than from the surface of the grains in order to provide better grain delineation.

Titanium and its solid solution alloys have been difficult to polish mechanically because the metal is quickly work-hardened yet at the same time it has a tendency to flow and hide the true grain structure in a manner somewhat analogous to the way in which a plastic will be deformed and hide a subsurface layer. Hand-polishing of such metal has been done but such is tedious for titanium and its alloys for the reason mentioned.

According to this invention a reagent has been discovered which is peculiarly suited to give good results with metallographic specimen of titanium and its alloys. The reasons therefor are unknown and the discovery of such has been empirical. Specifically, only one reagent formed from a number of old ingredients has been found satisfactory for the intended purpose. That one reagent includes 10 cc. of 48% C.P. hydrofluoric acid with 10 cc. of 69.3% of commercial nitric acid, 60 cc. of U.S.P. 3% hydrogen peroxide, and 30 cc. of distilled water. A better reagent composition has been found to result from the addition to the foregoing of 150 cc. of commercial glycerol having a specific gravity of 1.249. The best reagent for titanium metals and alloys is when 300 cc. of commercial ethylene glycol is added to the first mentioned combination of ingredients. In that first combination, plus or minus 5% by volume of each acid, the hydrogen peroxide and the distilled water constitute approximate limits for each of those components.

The time of immersion may vary depending upon the results desired, from 10 to 60 seconds. The work is then rinsed and dried. Having the polishing and etching bath at a slightly elevated temperature but not over about 200° F. will reduce the immersion time.

The functions of the various ingredients is not certain. The hydrofluoric acid is possibly the principal acid for attack upon the metal. The nitric acid and the hydrogen peroxide both cooperate in an oxidizing reaction. The distilled water serves as both a diluent and as a carrier or vehicle in producing a uniformly distributed polishing action. The ethylene glycol is believed to function as a carrier to insure uniformity in distribution of the polishing and etching action. The same may be said of the glycerol. Whatever the actions of these ingredients, it should be emphasized that their cooperative action results in the most satisfactory results with titanium solid solution alloys.

2

Among the advantages of this invention may be mentioned the provision of a polished light reflecting surface of titanium alloys at the same time a revealing etched surface is provided whereby the previous difficulties with mechanical polishing of this metal have been eliminated.

I claim:

1. A metallographic reagent for chemical polishing and simultaneously preferentially etching metallographic specimens of titanium and its alloys in solid solution whereby they are made ready for microscopic metallographic examination, said reagent consisting essentially of 10 parts by volume of 48% C.P. hydrofluoric acid, 10 parts by volume of commercial 69.3% nitric acid, 60 parts by volume of U.S.P. 3% hydrogen peroxide and 30 parts by volume of distilled water.
2. A chemical polishing reagent according to claim 1 having also at least 150 and not more than 300 parts by volume of one from a group consisting of ethylene glycol and glycerol.
3. A chemical polishing reagent according to claim 2 containing 150 parts by volume of glycerol.
4. A chemical polishing reagent according to claim 2 containing 300 parts by volume of ethylene glycol.
5. A process for preparing a specimen of titanium solid solution alloys for metallographic examination by reflected light from a specimen into a microscope which comprises chemically polishing said specimen to enhance reflectivity of light rays incident upon a surface of the specimen into a microscope, and simultaneously etching said surface of said specimen for delineation of grain boundaries during said polishing by reacting grain boundaries in said surface to the action of a reagent at a temperature of not over about 200° F. for not more than about one minute depending on the temperature of the reagent, and terminating said reaction by separating said surface from said reagent, when said reagent consists essentially of 10 parts by volume of 48% C.P. hydrofluoric acid, 60 parts by volume of U.S.P. 3% hydrogen peroxide, 10 parts by volume of commercial 69.3% nitric acid, and 30 parts by volume of distilled water.
6. A process according to claim 5 which includes in said reagent at least about 150 parts by volume and not more than about 300 parts by volume of one member of a group consisting of glycerol and ethylene glycol.
7. A process according to claim 5 in which said reagent includes about 150 parts by volume of glycerol.
8. A process according to claim 5 in which said reagent includes about 300 parts by volume of ethylene glycol.

## References Cited in the file of this patent

### UNITED STATES PATENTS

- |    |           |            |               |
|----|-----------|------------|---------------|
| 55 | 2,542,727 | Theuerer   | Feb. 20, 1951 |
|    | 2,606,960 | Little     | Aug. 12, 1952 |
|    | 2,687,345 | Murray     | Aug. 24, 1954 |
|    | 2,711,364 | Beach      | June 21, 1955 |
| 60 | 2,724,667 | MacPherson | Nov. 22, 1955 |
|    | 2,734,837 | Hands      | Feb. 14, 1956 |
|    | 2,828,192 | Langfield  | Mar. 25, 1958 |
|    | 2,876,144 | Bomberger  | Mar. 3, 1959  |

### FOREIGN PATENTS

- |    |         |               |               |
|----|---------|---------------|---------------|
| 65 | 753,158 | Great Britain | July 18, 1956 |
|    | 789,625 | Great Britain | Jan. 22, 1958 |

### OTHER REFERENCES

- 70 "New Etches for Germanium, by Ellis and Wolsky, from the Journal of Applied Physics, vol. 24, 1953; pages 1411 and 1412.